

## UNITED STATES PATENT OFFICE

2,515,147

PHOTOGRAPHIC DEVELOPER CONTAINING  
AN ARALKYLAMINE AND PROCESS OF  
DEVELOPMENTWilliam L. Wasley, Binghamton, N. Y., assignor  
to General Aniline & Film Corporation, New  
York, N. Y., a corporation of DelawareNo Drawing. Application August 26, 1947,  
Serial No. 770,750

12 Claims. (Cl. 95—88)

1

This invention relates to photographic developers and particularly to accelerators for photographic developers.

It is well-known that various amines, such as primary and secondary alkyl and alkylene amines containing from 3 to 7 carbon atoms, and heterocyclic amines, may be added to photographic black and white and color developing solutions for the purpose of increasing the rate of development. In other words, these amines accelerate the development so as to allow the developing agent to form the image (silver or color image) as rapidly as possible.

Although developing solutions containing such amines cut the developing time from about 20-30 minutes to 12-15 minutes, such a decrease is insufficient where large scale operations are involved, as in commercial processing where time is of the essence.

It is, therefore, an object of the present invention to provide a black and white and color developer having an increased rate of development so that the developing time is substantially decreased to less than half of the normal time.

Other objects will appear hereinafter.

These objects are accomplished by adding an aralkylamine to the usual black and white developer, and to a color-forming developer in which a primary aromatic amine is used as the developing agent. It has been found that in developing color images in multi-color photographic layers containing color-formers fast to diffusion, as disclosed in United States Patents 2,178,612; 2,179,228; 2,179,234; 2,179,238-9; 2,179,244; 2,186,719; 2,186,851-2; 2,186,732-3-4; 2,186,849; 2,200,306; 2,280,722; 2,292,575; 2,303,928 and 2,307,399, with a color developer containing an aralkyl amine, the developing time is cut from 20-30 minutes to 2-10 minutes. All of the layers are simultaneously developed, and the dye images formed are of excellent quality.

The developing time with black and white developers, for instance, solutions of hydroquinone and Metol and of hydroquinone and Elon, and the like, is also cut by more than half without causing fog when such solutions contain an aralkylamine.

The aralkylamines to be employed in accordance with the present invention are represented by the following general formulae:



and



2

wherein R is methyl or ethyl and n is a positive integer of from 2 to 3.

The following are examples of such aralkyl amines:

5



10



15



20



25



30

The amines are soluble in water and in alkaline developers, and may be used in specified amounts. The most useful concentrations in black and white developers range from about 1.0 cc. to about 10 cc. per liter. In color developers the most useful concentrations range from about 2.0 cc. to 7.0 cc. per liter. Concentrations greater than 7.0 cc. per liter of color developer have the tendency to distort the color balance of the color film.

As illustrative developing solutions containing such aralkylamines, the following are given:

## Example I

|                                |       |     |
|--------------------------------|-------|-----|
| Metol                          | grams | 0.8 |
| Sodium sulfite (anhydrous)     | do    | 45  |
| Hydroquinone                   | do    | 1.2 |
| Sodium carbonate (monohydrate) | do    | 8   |
| Potassium metabisulfite        | do    | 4   |
| Potassium bromide              | do    | 1.5 |
| $\alpha$ -Phenylethylamine     | cc    | 2.5 |
| Water to make                  | liter | 1.0 |

This tank developer gives, on development at 20° C. of the usual roll film, a soft negative in about 4-6 minutes after fixing and washing. The time required to develop a similar roll in the same developer and at the same temperature, but containing no  $\alpha$ -phenylethylamine, ranges from 15 to 20 minutes. Increasing the concentration of the  $\alpha$ -phenylethylamine to 5.0 cc. per liter effects a further decrease in time.

*Example II*

The following developer requires 30 minutes at 20° C. to give a satisfactory degree of color development with color paper:

|                                                      |       |     |
|------------------------------------------------------|-------|-----|
| Sodium hexametaphosphate                             | grams | 1.0 |
| Sodium bisulfite                                     | do    | 2.0 |
| N-N-bis(β-hydroxyethyl) - p-phenylenediamine sulfate | grams | 6.3 |
| Sodium carbonate                                     | do    | 100 |
| Hydroxylamine hydrochloride                          | do    | 1.0 |
| Potassium bromide                                    | do    | 1.0 |
| Water to make                                        | liter | 1.0 |

By the addition of 5 cc. of β-phenylethylamine to the foregoing developing solution, a color paper of excellent color rendition is developed in 5 minutes. Increasing the concentration of the amine further reduces the time of development.

The color paper (photographic multi-layer element) utilized in the foregoing example, consists of an integral tripack emulsion coated on either the usual paper base, or a clear cellulose acetate or nitrate film base, or in some cases an opaque white film base. Each of the emulsion layers is sensitized to one of the primary colors of light; namely, blue, green and red. The top layer is blue sensitive. A filter layer, yellow in color and blue absorbing, lies under the top layer. Below this filter layer, lies a green sensitive emulsion layer, and below this a red sensitive emulsion layer. Each of the three silver-halide emulsion layers contains dye-forming compounds which unite during the development of a silver image in an aromatic amine developing agent to form a dye with the oxidation product of the developing agent. As silver is also formed during development, it must be removed after color development by treatment in a bleach, followed by a bath of sodium thiosulfate, as is well-known to the art. A yellow dye is formed in the blue sensitive emulsion; a magenta dye is formed in the green sensitive emulsion; and a cyan dye is formed in the red sensitive emulsion. The combination of the dye images from these three printing primaries yields the color picture. Suitable methods for the preparation of multicolor emulsion layers have been described in the literature relating to color photography, and are, therefore, not described here.

*Example III*

The following developer requires 19 minutes at 20° C. to give a satisfactory degree of color development with color paper:

|                                                       |       |     |
|-------------------------------------------------------|-------|-----|
| Sodium hexametaphosphate                              | grams | 1.0 |
| Sodium bisulfite                                      | do    | 2.0 |
| N-ethyl-N-hydroxyethyl - p - phenylenediamine sulfate | grams | 6.7 |
| Sodium carbonate                                      | do    | 100 |
| Hydroxylamine hydrochloride                           | do    | 1.0 |
| Potassium bromide                                     | do    | 1.0 |
| Water to make                                         | liter | 1.0 |

By the addition of 2.5 cc. of α-phenylpropylamine to the foregoing developing solution, a color paper of excellent color rendition is developed in 4 minutes. Increasing the concentration of the amine to 6 cc. reduces the time of development to 2 minutes with the same results.

*Example IV*

The color developer of the preceding example with the addition of 5.0 cc. of α-phenylethylamine

developed a multi-layer color film sheet, of the reversal type and containing color-formers fast to diffusion, in 10 minutes at 20° C.; whereas without the α-phenylethylamine the time required to color develop the said film sheet is over 30 minutes.

The aralkylamines described herein have the advantage that they effect a simultaneous increase in contrast and greater reduction in developing time than other amines heretofore used for this purpose.

What I claim is:

1. An alkaline photographic developer for silver halide emulsions comprising an aqueous solution of a silver halide developing agent, an inorganic alkali and an aralkylamine selected from the class consisting of those corresponding to the following formulae:



25 and



wherein R is a group selected from the class consisting of methyl and ethyl groups, and n is a positive integer of from 2 to 3.

2. An alkaline photographic developer for silver-halide emulsions comprising an aqueous solution of a silver halide developing agent, an inorganic alkali and an aralkylamine characterized by the following formula:



3. An alkaline photographic developer for silver-halide emulsions comprising an aqueous solution of a silver halide developing agent, an inorganic alkali and an aralkylamine characterized by the following formula:



4. An alkaline photographic developer for silver-halide emulsions comprising an aqueous solution of a silver-halide developing agent, an inorganic alkali and an aralkylamine characterized by the following formula:



5. In the development of a photographic negative the step comprising the development of an exposed silver-halide emulsion in an aqueous solution of an alkaline silver halide developing agent, said solution containing an inorganic alkali and a developing accelerator selected from the

5

class consisting of aralkyl amines corresponding to the following formulae:



and



wherein R is a group selected from the class consisting of methyl and ethyl groups, and n is a positive integer of from 2 to 3.

6. In the development of a photographic negative the step comprising the development of an exposed silver-halide emulsion in an aqueous solution of an alkaline silver halide developing agent, said solution containing an inorganic alkali and a developing accelerator characterized by the formula:



7. In the development of a photographic negative the step comprising the development of an exposed silver-halide emulsion in an aqueous solution of an alkaline silver halide developing agent, said solution containing an inorganic alkali and a developing accelerator characterized by the formula:



8. In the development of a photographic negative the step comprising the development of an exposed silver-halide emulsion in an aqueous solution of an alkaline silver halide developing agent, said solution containing an inorganic alkali and a developing accelerator characterized by the formula:



9. A color-forming photographic developer comprising an aqueous solution of a primary aromatic amino developing agent, an inorganic alkali

6

and an aralkylamine selected from the class consisting of those corresponding to the following formulae:

5



and

10



15

wherein R is a group selected from the class consisting of methyl and ethyl groups, and n is a positive integer of from 2 to 3.

10. A color-forming photographic developer comprising an aqueous solution of a primary aromatic amino developing agent, an inorganic alkali and an aralkylamine characterized by the following formula:

25



30

11. A color-forming photographic developer comprising an aqueous solution of a primary aromatic amino developing agent, an inorganic alkali and an aralkylamine characterized by the following formula:

35



40

12. A color-forming photographic developer comprising an aqueous solution of a primary aromatic amino developing agent, an inorganic alkali and an aralkylamine characterized by the following formula:

45



WILLIAM L. WASLEY.

#### REFERENCES CITED

The following references are of record in the file of this patent:

#### UNITED STATES PATENTS

| Number       | Name           | Date          |
|--------------|----------------|---------------|
| 55 2,371,740 | Dearing et al. | Mar. 20, 1945 |
| 2,410,644    | Fierke et al.  | Nov. 5, 1946  |